

1

3,412,022

## SCROUPING AGENT FOR BULKED MULTI-FILAMENT YARNS

James E. Obetz, Chester, and Kimon C. Dardoufas, Colonial Heights, Va., assignors to Allied Chemical Corporation, New York, N.Y., a corporation of New York  
 No Drawing. Filed May 18, 1965, Ser. No. 456,820  
 15 Claims. (Cl. 252—8.7)

## ABSTRACT OF THE DISCLOSURE

The invention provides multi-filament bulked yarn of novel frictional characteristics, namely inter-filamentary slip-stick frictional force of 300–800 grams as the low up to 600–1200 grams as the high by the method of Schlatter et al., Textile Research Journal, volume XXIX, pages 200–210 (1959). These forces are imparted by applying to the filaments either a substituted diphenyl ether or a substituted naphthalene, containing at least one alkyl substituent and containing an acidic group in each of the rings of the ether or in the non-alkylated ring of the naphthalene. Preferably a yarn-to-metal lubricant is also applied to the yarn, especially a polyalkylene ether, imparting yarn-to-metal frictional force between 30 and 120 grams as measured by the above Schlatter et al. method.

This invention relates to new multi-filament textured or bulked yarns having exceptionally high inter-filamentary cohesive frictional properties. This invention, more particularly, relates to textured multi-filament yarns which in addition to having high inter-filamentary frictional properties have low metal-to-yarn frictional properties, the benefit of which will appear hereinafter. This invention further relates to a composition which imparts to multi-filament bulked yarns of any chemical composition high inter-filamentary frictional forces. This invention still further relates to a composition which in addition to imparting to bulked multi-filament yarns high inter-filamentary frictional properties enabling cohesiveness within the yarn also imparts to the yarn low metal-to-yarn frictional characteristics. This invention also relates to a process for applying the compositions to the yarn.

Bulked multi-filament yarns in many textile operations must be passed through various guides, needles and reeds in preparation of the end textile. For example, in the manufacture of say nylon carpets from bulked multi-filament yarn, it is the practice to pass the yarn through the eye of a metal tufting needle which acts much like the needle of an automatic sewing machine. The yarn is passed through at great speeds so that the maximum amount of carpet manufacture can be provided in a given time and hence the tufting needle works at a substantial speed. Since the yarn is composed of many individual filaments say about 200 there is a tendency for some of the filaments to stray from the yarn and separate out and loop around the tufting needle, and after several subsequent stitches, the entwined filaments pulls out the tufted stitch. This stitch "pulls out" and causes one or more of the following undesirable events, a defect in the carpet, tufting machine shutdown, and/or added cost for repairing the carpet defects. Hence, it is highly desirable to utilize, in many textile operations, a bulked multi-filament yarn which has cohesiveness within the yarn itself, i.e., a bulked multi-filament yarn which does not have individual filaments which tend to be separated from the yarn itself and to catch on or snag on guides, needles, reeds or the like. Such a multi-filament yarn would have high inter-filamentary frictional forces.

2

Another problem somewhat analogous to the above which is encountered with bulked multi-filament yarns in textile operations arises out of friction caused by the yarn being passed over or through the guides, needles, reeds, etc. This friction causes heat to be built up on the metal guides, needles, reeds, etc. The heat in turn causes certain individual filaments to stick and causes undesirable loops and filament separation along the yarn length. Alternately, filament sticking and filament separation can occur without heat build up due to frictional effects only. When either heat or frictional sticking of the filaments occurs, the individual filament can readily catch on the guide or the tufting needle and be separated from the yarn itself rendering much the same undesirable results discussed above. Hence, it is most desirable to utilize a bulked multi-filament yarn which has low metal-to-yarn frictional characteristics.

Various attempts have been made to solve the problems mentioned above particularly the first relating to the attainment of a coherent yarn free of filaments which tend to migrate freely from the confinement of the yarn bundle structure. One procedure aimed towards attainment of textured yarns by increase in inter-filamentary friction is disclosed in U.S. Patent 2,978,788 of Apr. 11, 1961 of Robert L. Keefe, Jr. entitled "Process for Treating Synthetic Yarn." The procedure therein disclosed involves application of a water sensitive size to the yarn e.g. an alkali metal salt of carboxymethyl cellulose, polyvinyl alcohol, drying the size, passing the dried yarn through a high velocity air jet to form a textured yarn, winding the textured yarn into a package and then subjecting the packaged yarn to warm humid air to reset the size and stabilize the filament convolutions. Such a procedure has obvious disadvantages and limitations. Notably, it involves costly multiple steps, requires control of humidity and the entanglements inserted limit the yarn "covering power" or pattern bloom which is highly desirable.

It is an object of this invention therefore to provide bulked, multi-filament yarns having high inter-filamentary frictional forces.

It is another object of this invention to provide bulked, multi-filament yarns having not only high inter-filamentary frictional forces indicative of their inter-filamentary cohesiveness, but also low metal-to-yarn frictional characteristics.

It is still another object of this invention to provide a scrouping agent, i.e. an agent which imparts inter-filamentary binding and cohesive forces, for bulked multi-filament yarns.

It is still another object of this invention to provide a scrouping agent composition which imparts to bulked multi-filament yarns low metal-to-yarn frictional properties.

A still further object of this invention is to provide a process for applying our scrouping agent composition to bulked multi-filament yarn.

These and other objects of our invention will become more apparent from the following description and claims.

According to our invention, we provide bulked yarns having high inter-filamentary frictional forces equivalent to a slip-stick frictional force low of 300 to 800 grams and a high of 600 to 1200 grams by applying thereto a solution of pH at room temperature between 2 and 12 of an aryl compound having the structural formula selected from the group consisting of



where A is an acid salt forming group, x is selected from the group consisting of hydrogen, nitrogen base radicals, and metal alkaline and alkaline earth metal atoms of the periodic chart of the elements having an atomic number not exceeding 56, preferably not exceeding 19, R is an alkyl group having between 1 and 30 carbon atoms inclusive, R' and R'' (which apply to I only) are independently selected from the group consisting of hydrogen, phenyl and phenoxy, and drying the so-treated yarn. The yarn has preferably applied thereto at least 0.2 to 2% by weight (dry basis) of this scrouping agent as an overfinish based on the weight of the yarns. An amount of scrouping agent of less than 0.2% by weight does not generally increase the inter-filamentary frictional forces while amounts greater than 2% by weight are unnecessary and hence represent merely added cost. Utilizing a yarn-to-metal lubricity additive as herein disclosed there is obtained, in addition to the high inter-filamentary frictional forces above, a low metal-to-yarn frictional force of between 30 and 120 grams.

The above aryl-ether (I) or alkyl naphthyl (II) compound, an ingredient of the scrouping agent is preferably water soluble at room temperature. However, other solvents can be used and in fact the overfinish can be applied using a dispersion consisting of the aryl compound and water or other liquid as vehicle. The scrouping agent (I) and alternately (II) is preferably applied to the yarn in a concentration of between 10% and 50% by weight. Use of a concentration of less than 10% necessitates application of a large amount of overfinish to provide the minimum preferred amount of scrouping agent on the yarn of 0.2%. On the other hand, the use of an aqueous solution of scrouping agent in concentration above 50% requires a higher degree of control in the application of the overfinish to the yarn so that no more than 2% by weight scrouping agent (on a dry basis) is applied to the yarn, which as indicated above, is the maximum desired amount of overfinish applied to the yarn.

The pH of the scrouping agent is important. A scrouping agent having a pH below 2 or above 12 will generally be too acid or basic as the case may be and will tend to attack the equipment used in applying the scrouping agent to the yarn or the yarn itself. Generally, we prefer to use a scrouping agent containing the above compounds I and II and having a pH at room temperature of between 4.5 and 9.5. A scrouping agent, according to our invention, with a pH below 4.5 tends to create corrosion problems for commercial operations while a scrouping agent of our invention with a pH above 9.5 tends to corrode aluminum type equipment which can be employed.

The aryl ether I or alternately the alkyl naphthyl compound II as depicted by the above formulae encompasses many specific ethers or alkyl naphthyl derivatives some of which are preferred over others, it being remembered that what is essential is that the compound be an aryl ether I or alternately an alkyl naphthyl II compound having at least one acid salt-forming group on each phenyl radical and an alkyl group on one phenyl radical. The specific acid salt-forming group (A) is not critical and can suitably be a sulfite, sulfate, hypophosphite, phosphate, phosphite, sulfonate or similar group or mixture thereof. We prefer the sulfonate radical as the acid-salt-forming group. Furthermore, the group—Ax can be the acid group itself or a salt thereof as x can be hydrogen, a nitrogen base radical, or a metal alkaline or alkaline earth atom having an atomic number not exceeding 56 preferably not exceeding 19. The term "nitrogen base radicals" includes ammonium or amine radicals. Hence,—Ax is the reaction product of the group A with compounds such as NH<sub>4</sub>OH or primary amines e.g. ethylamine or secondary amines e.g. dimethylamine. The term "alkaline or alkaline earth metal atoms of the periodic chart of the elements" as used herein refers to that periodic chart from Fundamental Chemistry, 2nd edition, by H. G. Deming, John Wiley, and Sons, Inc., as reprinted in the Handbook of

Chemistry by Lange, 10th edition, McGraw-Hill, 1961, pages 56-57. Hence, for compound I and alternately II the term includes lithium, rubidium, cesium, beryllium, sodium, magnesium, potassium, calcium, barium and strontium. We prefer for purposes of ease of procurement and water solubility to use a salt instead of the acid especially the sodium salt for obvious economic reasons. The alkyl group represented by R (I and alternately II) can vary in length from 1 to 30 carbon atoms and can be unsubstituted or substituted with halogens, carboxyl groups, by alcoholic OH groups and by pendent alkyl groups varying in length between 1 and 5 carbon atoms. R' and R'' applying to compound I can be either hydrogen atoms, phenyl group, or phenoxy groups. However, since there is no particular necessity in using the larger molecules they are not preferred. We have found that dodecylphenyl ether sodium disulfonate, whose structural formula is:



is an excellent aryl ether for use in the scrouping agent and that it performs excellently in the concentrations above mentioned to give the desired amounts of overfinish and accordingly is the desired aryl ether for our scrouping agent.

Alternately, we have found alkyl naphthalene sodium sulfonate, a preferred alkyl naphthyl derivative for our invention, can be employed in a similar manner to the aryl ether I above. The structural formula of the alkyl naphthalene sulfonate II is as follows:



40 A mixture of compounds having this structural formula is sold by Petrochemical Company under the trade name Petro-AG Special. This material is believed to be a 50-50 mixture of 1 methyl naphthalene 4 sodium sulfonate and 1-4 dimethyl naphthalene 5 sodium sulfonate.

45 As indicated above, the pH of the scrouping agent must be between 2 and 12 and is preferably between 4.5 and 9.5. Since the scrouping agent has acidic functions thereon it tends to be acid. However, the acidity can be adjusted with any suitable basic substance such as NaOH, KOH, NH<sub>4</sub>OH, H<sub>2</sub>NCH<sub>2</sub>CH<sub>2</sub>OH,



55 (CH<sub>3</sub>)<sub>2</sub>CHNH<sub>2</sub>. A preferred neutralizing or pH adjusting agent is a polyoxyethylene alkyl amine whose structural formula is



wherein R is alkyl and x and y are integers independently varying from 2 to 15 inclusive. An amine of this formula is manufactured under the trademark G3780-A, by Atlas Chemical Company.

70 The aqueous scrouping agent is applied to the bulked, multi-filament yarn by various methods preferably before thermal crimp removal. The mode of application can be by surface contact with either a metal or ceramic application roll; finish application by spraying or fogging of the scrouping agent onto moving yarn; by passage of the yarn through a slot with a thin film of the finish solution; and/or by direct contact by immersion

of the yarn in the scrouping agent. It is preferred to apply the scrouping agent prior to thermal crimp removal, since drying of the finish is accomplished simultaneously with crimp removal.

After the yarn is treated with the scrouping agent, it is dried. This operation can be performed by any conventional method as by passing the moist yarn through a heated chamber maintained at sufficient temperature to dry the yarn.

As a result there is provided a textured multi-filament yarn having high inter-filamentary frictional forces, to wit, a "slip-stick" frictional force low of 300 to 800 grams and high of 600 to 1200 grams. These inter-filamentary forces as reported are obtained by the "slip-stick" method of testing which is similar to the ASTM method and described by Schlatter, Olney and Baer in Textile Research Journal, vol. XXIX, pages 200-210, March (1959). Briefly, the yarn inter-filament frictional forces are determined as follows: using a Brush Tension analyzer Model ED-13-403-Brush Electronics Company, Cleveland, Ohio, the yarn to be tested is passed at a speed of 1 cm./minute over pulleys positioned so that the two strands under test which are twisted 1½ turn rubbing against each other at an imposed Helix arc of 360° with a positive tension of 400 grams. The frictional forces imposed are measured on the apparatus strain gage and recorded on a typical continuous recording chart. The chart frictional pattern shows a gradual increase in tension until the static friction is overcome. Then there is a rapid drop in tension until a level is reached where the dynamic friction overcomes this imposed tension. Thus the chart reads out in a "zig-zag" pattern showing a continuous series of low frictional measurement and gradual rise with sudden drops in friction, hence the name "slip-stick" friction.

The high "slip-stick" friction is the point at which static friction is overcome or as the cohesive forces in the practice of this invention are overcome and the low level being the point where the dynamic frictional forces are overcome as imposed by the cohesive forces by the scrouping agent employed in this invention.

The high "slip-stick" frictional properties imparted to bulked yarns by our scrouping agent are obtainable by all bulked yarns regardless of chemical composition, number of filaments, denier or similar factors. With yarn having such high frictional inter-filamentary properties, one can pass the yarn through guides and tufting needles at high speeds without any tendency of individual filaments to migrate freely from the confinement of the yarn bundle structure, thus enabling fast and easy production of bulked multi-filament yarn articles having excellent design patterns with the desired pattern definition and also exhibiting a high degree of "covering power" or "bloom."

The overfinish finish can be removed from the yarn readily in the normal scouring operating proceeding dyeing wherein the crimp or bulked effect returns to the yarn. No specific scouring agents are required to remove the overfinish as the overfinish is water soluble.

As indicated above, it is also desirable to provide a bulked, multi-filament yarn which not only has these high inter-filamentary frictional properties but also has low metal-to-yarn frictional characteristics. In order to provide this property, we have discovered that if a metal-to-yarn lubricity additive is employed in conjunction with our scrouping agent, that low metal-to-yarn frictional characteristics for multi-filament bulked yarns are obtained. The low metal-to-yarn frictional characteristics are provided to all types of bulked multi-filament yarns regardless of denier, number of filaments or chemical composition of yarn. The principal frictional characteristics of the yarn is a yarn-to-metal frictional force between 30 and 120 grams, believed by us to be novel for bulked multi-filament yarns. Where yarn-to-metal

frictional forces are referred to herein they were determined in a manner described by Schlatter in the same journal article as that which described yarn-to-yarn inter-filament frictional forces. The same Brush Tension analyzer is employed and the yarn is passed at a speed of 200 feet per minute with one turn over a polished stainless steel pin of surface finish of root mean square of 3.0 micro inches giving a metal-to-yarn angle of 360° against a floating pretension weight of 38 grams. The chart reading shows a constant tension which is a measurement of the yarn-to-metal frictional forces.

Suitable lubricity additives for our scrouping agent include in particular and preferably polyethers having the structural formula:



wherein  $R_1$  and  $R_3$  are independently selected from the group consisting of terminal hydroxyl groups, terminal hydroxyl groups esterified with acids of a chain length of 2 to 20 carbon atoms, and terminal hydroxyl groups etherified with alcohols of chain length of 2 to 20 carbon atoms,  $R_2$  is selected from the group consisting of hydrogen and methyl and  $n$  has a value of at least 3. These polyethers preferably have a molecular weight between 400 and 22,000 and suitably up to 30,000 and can be compounds such as polyethylene glycol or polypropylene glycol having an average molecular weight of 600, polyethoxylated fatty acids e.g. ethoxylated stearic acid or alcohols polyethoxylated with ethylene oxide e.g. ricinoleic acid glyceride (a chief ingredient of castor oil) polyethoxylated with ethylene oxide. In the latter case, the alcohols ethoxylated with ethylene oxide can have terminal hydroxyl groups and these terminal hydroxyl groups can be esterified with acids of a chain length between 2 and 20 carbon atoms inclusive.

When any of the above lubricity agents are present in the scrouping agent of this invention they should be present in an amount such that the ratio of scrouping agent to lubricity agent in parts by weight ranges from 1 to 8 parts scrouping compound per part lubricity agent, with smaller amounts of the lubricity agent permissible with a higher molecular weight (say above 10,000) of the lubricity agent. Except in the case of high molecular weight lubricity additives, smaller amounts of lubricity agent present in the scrouping agent do not generally impart the desired metal-to-yarn low frictional characteristics. Greater amounts of lubricity agent tend to yield poor package formation when the treated yarn is taken up on a package and/or deposit on guides and surfaces used in the processing. The lubricity agent is also removed from the yarn during the scouring operation and for this reason is desirably readily water soluble. However, it is not necessary that the lubricity agent be water soluble.

In order to more fully illustrate the nature of this invention and the manner of practicing the same, the following examples are presented. These are presented as preferred illustrative embodiments and are not to be construed as limitative of the scope of our invention. All values given, referring to quantities employed, unless otherwise stated, are by weight or parts by weight.

#### EXAMPLE I

A scrouping agent was made up as follows: 310 parts of a mixture of isomers of dodecyldiphenyl ether sodium disulfonate sold under the trademark Benax 2A1 by the Dow Chemical Company, believed to have the dodecyl group para the ether linkage and the  $SO_3Na$  groups on each phenyl group ortho or meta the ether linkage were added to 595 parts distilled water maintained under good agitation at a temperature of  $25^\circ C \pm 2^\circ C$ . To this scrouping agent was added 90 parts polyethylene glycol of average molecular weight 600 to be utilized in the scrouping agent as a yarn-to-metal lubricity agent. The aqueous solution was then neutralized with approximately

5 parts of a polyoxyethylene alkyl amine until a pH of 8.5 was obtained. The polyoxyethylene alkyl amine

acteristics were determined at 40% relative humidity, at a temperature of 76° C. and at a yarn angle of 360°.

TABLE I

| Percent Overfinish<br>Total Solids <sup>1</sup> | Twist Turns<br>Per Inch | Yarn Denier/<br>Number Filaments | Yarn-to-Yarn<br>Slip Stick<br>Friction <sup>2</sup> |      | Yarn-to-<br>Metal<br>Friction <sup>2</sup> | Crimps<br>Per Inch | Tufting<br>Performance | Cover of<br>Yarn and<br>Pattern<br>Definition |
|-------------------------------------------------|-------------------------|----------------------------------|-----------------------------------------------------|------|--------------------------------------------|--------------------|------------------------|-----------------------------------------------|
|                                                 |                         |                                  | Low                                                 | High |                                            |                    |                        |                                               |
| Control.....                                    | 0                       | 0.....                           | 3600/210                                            | 270  | 460                                        | 42                 | 12-13                  | Poor.....                                     |
| This example.....                               | 0.8                     | 0.....                           | 3600/210                                            | 370  | 670                                        | 80                 | 12-13                  | Satisfactory.....                             |
| Control.....                                    | 0                       | 1/4 S.....                       | 3600/210                                            | 240  | 480                                        | 38                 | 12-13                  | Poor.....                                     |
| This example.....                               | 0.9                     | 1/4 S.....                       | 3600/210                                            | 450  | 750                                        | 85                 | 12-13                  | Good.....                                     |
| Control.....                                    | 0                       | 1/4 S.....                       | 3150/210                                            | 250  | 460                                        | 34                 | 13-14                  | Fair.....                                     |
| This example.....                               | 1.3                     | 1/4 S.....                       | 3150/210                                            | 500  | 810                                        | 65                 | 13-14                  | Excellent.....                                |

<sup>1</sup> Percent Overfinish per unit, weight of yarn.

<sup>2</sup> Friction is the frictional forces in grams using the above described method.

utilized was one manufactured by the Atlas Chemical Company under the trademark Atlas G3780A and having roughly the following empirical formula:



wherein  $x$  and  $y$  in the formula are independently integers varying between 2 and 15 inclusive.

The aqueous scrouping agent solution was then placed in a trough in which rotated 12" length stainless steel application roller, 4" in diameter, over which passed 20 ends of "O" twist yarn of 3,600 denier, 210 filament nylon crimped carpet yarn at a rate of 800 ft. per minute. The speed of the stainless steel application roller was maintained at 30 r.p.m. to apply approximately 0.80% by weight (on a dry basis) overfinish to the bulked yarn. A tangential contact angle of between 1 and 2° for a distance of 1/8" to 1/4" on the stainless steel roller face at a tension of between 200 and 500 grams per end of 3,600 denier yarn was maintained. The scrouping agent applied immediately after crimping and prior to thermal crimp removal taking advantage of the heat applied during crimp removal to dry the applied overfinish.

A control yarn of the same denier and number of filaments was treated in the same manner with the exception of treatment with the scrouping agent. Several controls having various twists were also treated in the manner of the first mentioned control. Accordingly, yarns having the same twist and denier as their respective control were treated with the scrouping agent in the man-

15 The yarn coated with finished as above described was employed in making loop pile tufted nylon carpets having six tufts per inch and 20 ounces of fiber per square yard carpet, employing woven jute backing of 12 ounces per square yard. The tufting needle had an oval shaped eye, 1 1/4" side and 1/4" wide operated at a rate of 520 tufts per minute. As a measure of runnability of the yarn through the tufting needle the number of stoppages or quality defects due to the behavior of the yarn was counted per square yard of tufted carpet. Generally speaking, good operation of carpet tufting operations is said to exist when there are less than 2.5 occurrences of stoppages or defects per 25 square yard carpet. Greater occurrence of stoppages are indicative of fair-to-poor runnability of the yarn indicating either high yarn-to-metal frictional characteristics or low inter-filamentary frictional properties of the yarn itself.

20 The samples of the tufted carpet were scoured at 212° F. and rope dyed in a beck. The standard latex dispersion was subsequently applied to the backings of the samples. 25 The carpet samples were test evaluated for covering power by visual determination of whether the white colored carpet backing could be seen through the pile surface when viewed from above. The "pattern definition" was ascertained by visual observation of pattern uniformity and precision. For purposes of comparison, control trials 30 were carried out using carpets of identical construction made from identically treated yarn except for treatment with the scrouping agent to provide an overfinish on the yarn. Experimental results and observations are presented 35 in Table II below.

TABLE II

| Trial  | Type Trial                                                                                                                                              | Twist<br>Turns<br>Per<br>Inch | Percent<br>Overfinish<br>Added <sup>1</sup> | Sample<br>Tufting<br>Defects<br>25/yds. <sup>2</sup> | Tufting<br>Performance             | Carpet Quality      |                                     |
|--------|---------------------------------------------------------------------------------------------------------------------------------------------------------|-------------------------------|---------------------------------------------|------------------------------------------------------|------------------------------------|---------------------|-------------------------------------|
|        |                                                                                                                                                         |                               |                                             |                                                      |                                    | Quality of<br>Cover | Quality of<br>Pattern<br>Definition |
| 1..... | Control.....                                                                                                                                            | 1/4                           | 0                                           | 196                                                  | Poor.....                          | Non-uniform.....    | Poor-Rough.....                     |
| 2..... | Yarn treated as above with composition of this example.....                                                                                             | 1/4                           | 0.8                                         | 82                                                   | Good.....                          | Good.....           | Good.....                           |
| 3..... | Dodecyldiphenyl ether sodium disulfonate (3 parts);<br>polyethylene glycol 1,000 (6 parts); sorbitol (2.5 parts),<br>with commingled yarn. <sup>4</sup> | 1/3                           | 1.5                                         | 37                                                   | Fair (deposits) <sup>3</sup> ..... | Fair.....           | Fair.....                           |
| 4..... | Yarn treated as above with composition of this example<br>and commingled yarn. <sup>4</sup>                                                             | 1/3                           | 1.8                                         | 15                                                   | Very good.....                     | Good.....           | Good.....                           |
| 5..... | Yarn treated as above with composition of this example.....                                                                                             | 1/4                           | 0.4                                         | 114                                                  | Fair.....                          | Fair.....           | Fair.....                           |
| 6..... | .....do.....                                                                                                                                            | 1/4                           | 0.8                                         | 92                                                   | Good.....                          | Good.....           | Good.....                           |
| 7..... | .....do.....                                                                                                                                            | 1/4                           | 1.5                                         | 45                                                   | do.....                            | do.....             | Do.....                             |

<sup>1</sup> Overfinish per unit, weight of yarn.

<sup>2</sup> Adjustment of experimental tufting was made to produce increased defects corresponding to a normal commercial tufting multiplied by a factor of 35. Therefore to interpret the above tufting control data to a commercial performance the tufting defect data should be divided by 35.

<sup>3</sup> Deposits; otherwise, performance was good.

<sup>4</sup> Commingled yarn is yarn having a high degree of inter-filamentary coherency so that it is readily runnable over and through guides, needles and reeds involved in textile operation. It is produced in accordance with U.S. application Ser. No. 535,480 of Fred W. Le Noir, entitled "Commingled Crimped Yarn," filed Mar. 18, 1966.

65 The above described applying varying amounts of overfinish to the yarn. The yarn-to-yarn slipstick frictional forces of all yarns both treated and untreated was determined as well as the yarn-to-metal frictional forces of each yarn. The results of these determinations are set forth in Table I below. By reference to this table, it can be noted the dramatic and significant effect upon the frictional properties of yarn as compared to conventional crimped yarns in which no overfinish was applied by use of the scrouping agent. These beneficial frictional properties are imparted by the scrouping agent of our invention. In Table I below the yarn frictional char-

70 According to the invention commingled yarn is produced by continuously advancing successive lengths of a crimped multi-filament yarn at a tension of between .003 and .015 gram per denier through a region of confinement, contacting the yarn in the region of confinement with a gas at a pressure below 40 p.s.i.g., causing at least 90% of the gas to flow in contact with the yarn and in a path counter-current to the direction of the yarn travel, and causing the yarn in the course of its entering and exiting from the region of confinement to follow essentially a straight line path. The commingled yarn has 75 spaced zones of comminglement and non-commingle-

ment. In the zone of comminglement unlike the interlaced yarn structures of the prior art, there are essentially no peripheral filaments which completely wrap about the yarn bundle or about major portions of the yarn bundle. The commingling instead involves filament inter-action affecting only closely adjacent filaments without extensive transmission of isolated effects across the diameter of the yarn bundle or along the length of the yarn. Hence, the forces which tend to draw the bundle together and thereby maintain its integrity or cohesiveness are of lesser mechanical stability than interlaced configurations heretofore provided wherein peripheral filaments encircle or otherwise interact with the entire bundle of major portions thereof.

#### EXAMPLES 2-12

The same procedures, as in Example 1, was employed and the frictional properties of various additives, which were evaluated, were compared with the product of this invention. All yarns employed were  $\frac{3}{4}$  turn twist nylon carpet yarns. The results are tabulated in Table III.

15 20 The terms and expressions which have been employed are used as terms of description and not of limitation,

TABLE III

| Ex.<br>No. | Component A Name                             | Component B Name                                   | Weight<br>Percent<br>A on<br>Yarn | Weight<br>Percent<br>B on<br>Yarn | Yarn-to-Yarn Slip |                | Grams<br>Yarn-<br>to-Metal<br>Friction | Tufting<br>Performance      | Cover and<br>Pattern<br>Definition |
|------------|----------------------------------------------|----------------------------------------------------|-----------------------------------|-----------------------------------|-------------------|----------------|----------------------------------------|-----------------------------|------------------------------------|
|            |                                              |                                                    |                                   |                                   | Low,<br>Grams     | High,<br>Grams |                                        |                             |                                    |
| 2          | Dodecyldiphenyl Ether<br>Sodium Disulfonate. | Polyethylene Glycol 600,<br>M.W. 600 $\pm$ 30.     | 0.33                              | 0.22                              | 450               | 750            | 85                                     | Good.....                   | Excellent.                         |
| 3          | do                                           | do                                                 | 0.17                              | 0.10                              | 370               | 670            | 80                                     | Fair.....                   | Good.                              |
| 4          | do                                           | do                                                 | 0.60                              | 0.35                              | 460               | 755            | 90                                     | Good.....                   | Excellent.                         |
| 5          | do                                           | Polyethylene Glycol 400,<br>M.W. 400 $\pm$ 20.     | 0.64                              | 0.37                              | 560               | 700            | 130                                    | Fair.....                   | Good.                              |
| 6          | do                                           | Polyethylene Glycol<br>1,000, M.W. 1,000 $\pm$ 50. | 0.49                              | 0.35                              | 460               | 745            | 135                                    | do.....                     | Fair.                              |
| 7          | Dimethyl Hydantoin<br>Formaldehyde Resin.    | Polyethylene Glycol 1,000.                         | 0.4                               | 0.4                               | 305               | 580            | 90                                     | Poor.....                   | Poor.                              |
| 8          | Polyvinyl Alcohol <sup>1</sup>               | Polyethylene Glycol 600,<br>M.W. 600 $\pm$ 30.     | 0.6                               | 0.35                              | 270               | 545            | 60                                     | do.....                     | Do.                                |
| 9          | Dodecyldiphenyl Ether<br>Sodium Disulfonate. | Castor Oil+200 Moles<br>Ethylene Oxide.            | 0.48                              | 0.24                              | 460               | 650            | 130                                    | Fair-Good....               | Fair-Good.                         |
| 10         | do <sup>3</sup>                              | Polyethylene Glycol<br>1,000, Sorbitol.            | 0.3                               | 0.6/25                            | 540               | 670            | 90                                     | Fair-Good <sup>2</sup> .... | Do.                                |
| 11         | do                                           | Polyethylene Glycol 20M,<br>M.W. 20,000 $\pm$ 100. | 0.79                              | 0.11                              | 612               | 1,104          | 105                                    | Good.....                   | Good.                              |
| 12         | Alkyl Naphthalene<br>Sodium Sulfonate.       | Polyethylene Glycol 20M,<br>M.W. 20,000 $\pm$ 100. | 0.88                              | 0.12                              | 400               | 1,106          | 85                                     | do.....                     | Excellent.                         |

<sup>1</sup> A dispersing agent was added.

<sup>2</sup> Powdering.

<sup>3</sup> 3 parts.

#### EXAMPLES 13-19

The same procedure, as in Example 1, was employed except that the scrouping agent was an alkyl naphthalene sodium sulfonate supplied by Petrochemical Company under the trade name Petro-AG Special.

The weight concentration of the scrouping agent and various lubricating agents which were evaluated were varied and compared with the product of this invention as to frictional properties and tufting quality and performance. All yarns employed were  $\frac{3}{4}$  turn twist nylon carpet yarns.

The results are tabulated in Table IV.

45 and there is no intention, in the use of such terms and expressions, of excluding any equivalents of the features shown and described or portions thereof, but it is recognized that various modifications are possible within the scope of the invention claimed.

We claim:

50 55 1. A multi-filament bulked yarn having a slip-stick frictional force low of 300 to 800 grams and a high of 600 to 1200 grams, said yarn being coated with an overfinish in an amount of from 0.2% to 2% of the total weight of the yarn on a dried weight basis, said overfinish having a pH at room temperature of between about 2 and

TABLE IV

| Ex.<br>No. | Component A Name                       | Component B Name                                   | Weight<br>Percent<br>A on<br>Yarn | Weight<br>Percent<br>B on<br>Yarn | Yarn-to-Yarn Slip |                | Grams<br>Yarn-<br>to-Metal<br>Friction | Tufting<br>Performance | Cover and<br>Pattern<br>Definition |
|------------|----------------------------------------|----------------------------------------------------|-----------------------------------|-----------------------------------|-------------------|----------------|----------------------------------------|------------------------|------------------------------------|
|            |                                        |                                                    |                                   |                                   | Low,<br>Grams     | High,<br>Grams |                                        |                        |                                    |
| 13         | Alkyl Naphthalene<br>Sodium Sulfonate. | Polyethylene Glycol 20M,<br>M.W. 20,000 $\pm$ 100. | 0.88                              | 0.12                              | 400               | 1,106          | 85                                     | Good.....              | Excellent.                         |
| 14         | do                                     | do                                                 | 0.14                              | 0.02                              | 440               | 594            | 35                                     | Fair.....              | Fair.                              |
| 15         | do                                     | do                                                 | 0.66                              | 0.09                              | 432               | 804            | 90                                     | Good.....              | Excellent.                         |
| 16         | do                                     | Polyethylene Glycol 600,<br>M.W. 600 $\pm$ 30.     | 0.62                              | 0.08                              | 440               | 740            | 75                                     | do.....                | Good.                              |
| 17         | do                                     | 2-pyrrolidone                                      | 0.84                              | 0.12                              | 588               | 1,058          | 190                                    | Poor.....              | Poor.                              |
| 18         | do                                     | CF-32 <sup>1</sup>                                 | 0.70                              | 0.40                              | 490               | 713            | 110                                    | Fair.....              | Fair.                              |
| 19         | do                                     | PVP-618 (polyvinyl-<br>pyrrolidone).               | 0.80                              | 0.20                              | 396               | 1,078          | 130                                    | Poor.....              | Do.                                |

<sup>1</sup> CF-32.—Amine polyglycol condensate supplied by Rohm & Haas.

70 75 It is readily seen from the foregoing that we have provided new multi-filament bulk yarns having exceptionally high inter-filamentary frictional forces together with, if desired, low metal-to-yarn frictional characteristics particularly useful in carpet manufacture and the like. The yarns that we have provided are believed by

about 12 and consisting essentially of an aryl compound of the formula selected from the group consisting of:



wherein:

A is an acid salt-forming substituent selected from the group consisting of sulfate, sulfite, phosphate, phosphite, hypophosphite, and sulfonate substituents; x is a substituent selected from the group consisting of hydrogen substituent, alkali metal and alkaline earth metal of atomic number not exceeding 56, and nitrogen base selected from the group consisting of ammonium, mono-lower-alkylammonium, and di-lower-alkylammonium;

R is an alkyl group of between about 1 carbon atom and about 30 carbon atoms inclusive; and

R' and R'' are each independently selected from the group consisting of hydrogen, phenyl, and phenoxy.

2. A multi-filament bulked yarn according to claim 1 wherein said aryl compound has the formula:



3. A multi-filament bulked yarn according to claim 1 wherein said aryl compound has the formula:



4. A yarn according to claim 1 wherein the over-finish is present in an amount between 0.2 and 2% by weight of the total weight of the yarn on a dried weight basis.

5. A multi-filament bulked yarn according to claim 4 wherein A is  $-\text{SO}_3^-$ .

6. A multi-filament bulked yarn according to claim 4 wherein  $-\text{Ax}$  is  $\text{SO}_3\text{Na}$ .

7. A multi-filament bulked yarn according to claim 4 wherein said aryl compound has the formula:



8. A process for imparting high inter-filamentary forces to bulked multi-filament yarn which process comprises applying to said yarn, from an aqueous solution having a pH at room temperature of between about 2 and about 12, an aryl compound of the formula selected from the group consisting of:



wherein:

A is an acid salt-forming substituent selected from the group consisting of sulfate, sulfite, phosphate, phosphite, hypophosphite, and sulfonate substituents; x is a substituent selected from the group consisting of hydrogen, alkali metal and alkaline earth metal of atomic number not exceeding 56, and nitrogen base selected from the group consisting of ammonium, monoalkylammonium, and dialkylammonium;

R is an alkyl group of between about 1 carbon atom and about 30 carbon atoms inclusive; and

R' and R'' are each substituents independently selected from the group consisting of hydrogen, phenyl, and phenoxy substituents,

said aryl compound being applied to the yarn in an amount of from 0.2% to 2% of the total weight of the yarn on a dried weight basis to impart to said yarn a slip-stick frictional force low of 300-800 grams and a high of 600-1200 grams.

9. A process according to claim 8 wherein said aryl compound has the formula:



10. A process according to claim 8 wherein said aryl compound has the formula:



11. A process according to claim 8 wherein said atomic number does not exceed 19.

12. A process according to claim 8 wherein A is  $-\text{SO}_3^-$ .

13. A process for imparting to bulked multi-filament yarn high inter-filamentary frictional forces according to claim 8 wherein a mixture of 1-methyl-naphthalene-4-sodium sulfonate with 1,4-dimethyl-naphthalene - 5 - sodium sulfonate is employed as the aryl compound.

14. A process according to claim 8 wherein said aqueous solution has a pH of between 4.5 and 9.5.

15. A process according to claim 14 wherein said acid salt-forming group, A, is  $\text{SO}_3^-$  and said aqueous solution contains a polyether lubricity additive of the formula:



wherein  $\text{R}_1$  and  $\text{R}_3$  are independently selected from the group consisting of terminal hydroxyl groups, terminal hydroxyl groups esterified with acids of a chain length of 2 to 20 carbon atoms, and terminal hydroxyl groups etherified with alcohols of chain length of 2 to 20 carbon atoms,  $\text{R}_2$  is selected from the group consisting of hydrogen and methyl and  $n$  has a value of at least 3 and the molecular weight of said polyether additive is between 400 and 22,000; the non-aqueous ingredients of said solution consisting essentially of said aryl compound and said polyether; the concentrations in said solution and the amount of said solution applied to said yarn being adjusted to provide from 0.2% to 2% by weight of said non-aqueous ingredients on a dry basis on the yarn and to provide in said solution between about 1 and about 8 parts by weight of said aryl compound per part by weight of said polyether.

#### References Cited

#### UNITED STATES PATENTS

2,854,477 9/1958 Steinhauer ----- 260—612

LEON D. ROSDOL, Primary Examiner.

S. D. SCHWARTZ, Assistant Examiner.